

March 18, 1941.

W. J. SWEENEY

2,235,124

VOLTOLIZATION OF HYDROGENATED PRODUCTS

Filed Dec. 30, 1937



William J. Sweeney Inventor  
By *P. Young* Attorney

## UNITED STATES PATENT OFFICE

2,235,124

## VOLTOLIZATION OF HYDROGENATED PRODUCTS

William J. Sweeney, Elizabeth, N. J., assignor to  
Standard Oil Development Company, a corpora-  
tion of Delaware

Application December 30, 1937, Serial No. 182,440

## 1 Claim. (Cl. 204—168)

The present invention relates to a process of producing improved lubricating materials and the products thereof. It relates to the production of oxidation resistant lubricating oils having high viscosity and high viscosity indexes. It particularly relates to the process of producing these materials from initial materials which heretofore have had relatively little value and which are produced in lubricating oil solvent treating processes. These initial materials are secured from the extract when solvent extracting agents having a preferential selectivity for compounds having a lower ratio of hydrogen to carbon, as compared to compounds having a higher ratio of hydrogen to carbon, are employed. If solvents are employed which have a preferential selectivity for compounds having a higher ratio of hydrogen to carbon, as compared to compounds having a lower ratio of compounds to carbon, the initial materials are found in the raffinate. The process of the present invention segregates these initial aromatic type materials and hydrogenates them under suitable non-cracking conditions and then voltolizes the hydrogenated product.

The invention may be readily understood by reference to the attached drawing illustrating one modification of the invention. Suitable material for the solvent treatment step is fed into solvent treating unit 1 through feed line 2 where it intimately contacts a solvent. In the flow plan illustrated, a solvent having a preferential selectivity for compounds having a lower ratio of hydrogen to carbon is employed as, for example, phenol. This solvent is fed into solvent treating unit 1 by means of feed line 3. The raffinate or the treated material is removed through line 4 while the solvent containing the extract is removed through line 5 and then fed into the solvent recovery unit 6. In this unit the solvent is removed from the extract by known methods and taken off by means of line 3. The extract is removed from the solvent recovery unit 6 by means of line 7 and led into the hydrogenation unit 8 in which it is hydrogenated by means of hydrogen fed into said unit by means of line 9. The hydrogenated extract is removed through line 10 and led into voltolization unit 11 in which it is treated with the silent electric glow discharge in order to secure the product desired. The finished voltolized hydrogenated extracted product is removed through line 12 and may be used as such or may be segregated into a particular fraction desired by suitable known means.

55 The initial materials suitable for solvent ex-

tracting may vary widely. It is preferred, however, to use petroleum hydrocarbons as, for example, light, middle or heavy mineral oils, naphtha, gas oils, burning oils and the like. Preferred materials are petroleum hydrocarbons 5 boiling in the lubricating oil range. Preferred extracts are those which are secured in the process of refining lubricating oils by solvent treating methods. In this process lubricating oils, usually paraffinic in nature, having gravities A. P. I. from 25 to 35 and a flash of from 300° F. to 500° F. and higher and a viscosity Saybolt of from 200 at 100° F. to 140 at 210° F. are fed into a solvent treating unit. This unit may be a batch treating apparatus but is preferably a continuous treating plant having one or more individual units. In this unit the feed materials are intimately contacted with solvent and the desirable saturated paraffinic type of materials are separated from the relatively unsaturated and aromatic type of materials. Solvents having a preferential selectivity for the former type of materials as, for example, liquid normally gaseous hydrocarbons, may be employed as, for example, liquid propane and butane. 25 Solvents having a preferential selectivity for compounds having a lower ratio of hydrogen to carbon may be employed as, for example, furfural, liquid sulphur dioxide, phenol, nitrobenzene, cresylic acid, acetonitrile, aniline, acetone, 30 and the like.

The conditions of solvent extracting are adjusted for the particular feed stock being treated, the solvent being used and the desired quality and yield of the products. The temperature is 35 preferably in the range from —20° F. to 250° F. and the ratio of the volume of solvent to volume of oil treated is preferably from  $\frac{1}{2}$  to 10. For example, when phenol is employed, the phenol to oil ratio varies from 100 to 200% depending upon the stock handled and the desired quality of the treated oil. The temperature employed is in the range from 100 to 250° F. In general higher temperatures and higher ratios of phenol to oil results in an improvement in 45 quality of the raffinate and with a higher yield of the extract. For each particular stock treated, optimum conditions of temperature and solvent oil ratio must be determined in order to secure the desired products.

50 The spent solvent containing the extract may be separated from the raffinate either by gravity settling or by other means as, for example, centrifuging. If a solvent of the type of phenol is employed, the spent solvent is then taken to a 55

- solvent recovery plant in which the solvent is removed from the extract. The yield of the extract may vary widely, depending upon the conditions under which the initial materials are treated.
- 5 Preferred materials are secured by extracting petroleum lubricating hydrocarbons with a phenol under conditions whereby the spent phenol contains approximately 10 to 30% extract. The extract after the removal of the solvent
- 10 is then led to a hydrogenation unit in which it is hydrogenated under suitable conditions. It is desired to hydrogenate the extract under substantially non-cracking conditions and to secure a substantially saturated product. This is secured by hydrogenating at temperatures below 15 750° F. in the general range in which there is little or no decomposition of the oil. The temperatures and pressures employed depend particularly upon the material to be treated, as well
- 20 as the catalyst employed and on the duration of the treatment. Thus temperatures up to 850° may be employed providing the duration of the treatment is adjusted so that substantially no cracking occurs. The pressures employed are
- 25 preferably in the range of from 10 to 20 atmospheres although pressures as high as 100 to 200 atmospheres may also be employed. The hydrogenation of the oil under conditions to secure substantially no cracking and to secure substantially a saturated product is very important. This is necessary in order to secure a product which is susceptible to subsequent voltolization and is necessary in order to give desirable voltolization products.
- 30 35 The hydrogenated product is then subjected to voltolization. The process of voltolization consists in subjecting material to the effect of the high tension silent electric discharge, commonly known as the glow discharge. The process of voltolization varies from .001 mm. to .01 atmosphere, .5 atmosphere, or even as high as .8 atmosphere and higher. It is preferred, however, to have the pressure below one atmosphere. The voltages used are preferably in the range from
- 4,000 to 10,000 volts although voltages as high as 20,000 or 50,000 may be utilized, providing suitable dielectrics are available. The frequency of the alternating current may be as low as 60 cycles and may be as high as 1,200 to 10,000 cycles or 5 more. In the voltolization operation, it is preferred to provide external cooling means in order to keep the temperature sufficiently low in order that the quality of the products may not be lowered. This is necessary since the heat of the reaction is frequently sufficient to raise the temperature of the mixture to 300° C. and higher. It may be desirable to voltolize at temperatures below 0° C. as, for example, at a temperature as low as -40° C.
- 10 15 20 25 30 35 40
- The voltolization operation is continued for a time sufficient to secure a product having the desired viscosity. Preferred products are those having viscosities in the range from 100 to 8,000 Saybolt at 210° F.
- The above invention is not to be limited by any theory or method of operation but only by the following claim in which it is desired to claim all novelty in so far as the prior art permits.
- I claim:
- The process which comprises treating a petroleum lubricating oil fraction having an A. P. I. gravity of 25 to 35, a flash of from 300° F. to 500° F. and a Saybolt viscosity from 200 seconds at 100° F. to 140 seconds at 210° F. with a selective solvent adapted to separate compounds having a lower ratio of hydrogen to carbon from compounds having a higher ratio of hydrogen to carbon, separating the resultant oil fractions, hydrogenating the fraction having the lower ratio of hydrogen to carbon and which is substantially free from paraffinic hydrocarbons, under substantially non-cracking conditions to secure substantially a saturated oil, and then voltolizing the resultant hydrogenated oil to a viscosity in the range of 100 to 8,000 seconds Saybolt at 210° F.

WILLIAM J. SWEENEY.